# EUROPEAN PATENT SPECIFICATION

(11) **EP 0 256 555 B1**
(45) Date of publication and mention of the grant of the patent: **21.10.1992**
(21) Application number: 87111982.2
(22) Date of filing: 18.08.1987
(51) Int. Cl.: C22C 1/10, C22C 32/00

(54) **Dispersion strengthened alloys**
Dispersionsverstärkte Legierungen
Alliages renforcés par dispersion

(30) Priority: 18.08.1986 US 897745
(43) Date of publication of application: 24.02.1988
(73) Proprietor: Inco Alloys International, Inc., Huntington West Virginia 25720 (US)
(72) Inventor: Benn, Raymond Christopher, Huntington, W VA 25705 (US); Fischer, John Joseph, Huntington, W VA 25701 (US); Smith, Gaylord Darrell, Huntington, W VA 25705 (US)
(74) Representative: Greenstreet, Cyril Henry

(56) References cited:
- EP-A- 0 091 260
- AU-B- 19 134
- US-A- 3 992 161
- US-A- 4 402 746

## Description

The present invention is directed to dispersion-strengthened (DS) alloys, and more particularly to oxide-dispersion strengthened (ODS) iron-base alloys which manifest an exceptional degree of resistance to oxidation at temperatures as high as 1300°C (approx. 2400°F) whereby the alloys are useful in the production of advanced aircraft gas turbine engine components and in demanding industrial applications.

Except where otherwise specified, all percentages herein are by weight. All percentages by weight and by volume are based on the total weight or volume of the alloy, respectively.

In U.S. Patent 3,992,161 ('161) ODS iron-chromium alloys are described as having very good oxidation resistance coupled with high-strength at elevated temperatures. The results set forth therein reflect a decided improvement over iron-chromium alloys produced by the more conventional melt/ingot processing practices. More specifically, it was disclosed that the ODS alloys could be produced by the now well known Mechanical Alloying process, a technology developed nearly twenty years ago and described in such U.S. Patents as 3,591,362 and 3,837,930.

Notwithstanding the virtues of the '161 alloys such materials have been found wanting in certain aerospace and industrial environments. By way of explanation, though the '161 ODS material (commercially containing about 20% chromium, 4.5% aluminum) exhibits good corrosion and oxidation resistance at, say, up to 1200°C, it is prone to undergo premature slagging attack (formation of low melting point phases/compounds through a chemical reaction with corrosive deposits from and/or the environment per se) and/or accelerated attack upon exposure at higher temperatures after short intervals of time, the failure being of the catastrophic type. In this connection, accelerated oxidation may be considered as the rapid mass change of an alloy by oxidation. The mass change is virtually always dramatically positive if all the oxide is collected and weighed. In undergoing the ravages occasioned by such attack the alloy surface converts to friable iron oxide and iron-chromium spinels.

For example, burner cans in aircraft gas turbine engines of advanced design are currently intended for use at increasingly higher operating temperatures, i.e., about 1250°C (2308°F), and above, e.g., 1300°C (2372°F). Similarly, industrial applications involving intimate contact with such aggressive corrosives as flue dust, fly ash, molten glass, etc. require more oxidation and/or corrosion-resistant materials.

Apart from the above, what is also required for such applications is a material which offers in addition to high strength at operating temperatures, including stress-rupture and tensile characteristics, sufficient fabricability that it can be formed into flat rolled products such as sheet, strip, etc, which product forms can be formed into tubing, rings, canisters and other shapes. With-out fabricability the utility of an ODS material is significantly diminished.

Apart from '161 reference also might be made to the work of Kornilov, "Aluminum in Iron and Steel" by S.C. Case and K.R. Van Horn, John Wiley and Sons (1953). Kornilov studied the effect of up to 10% aluminum and up to 65% chromium on scaling losses in both cast and wrought Fe-Cr-Al alloys. Aluminum benefited scaling resistance but seemingly there was little benefit conferred by chromium beyond the 25% level at 1100-1400°C. Nothing in the Kornilov investigation involved fabricability of an ODS product or manufacture of sheet.

R. Allen and R. Perkins (in a contract report for the Naval Air Systems Command, May 1973) investigated ODS iron-chromium-aluminum-yttrium alloys with 16-25% chromium at an aluminum level of 5.7-6.0% versus conventional wrought and cast 25% Cr/4% Al and 15% Cr/4% Al alloys. It was indicated that such alloys could be extruded but nothing was given in terms of fabricability and the production of, say, the important sheet product form.

It has now been found that certain ODS iron-base compositions having special and correlated percentages of chromium and aluminum and a refractory dispersoid afford an outstanding degree of resistance to oxidation/corrosion such that the alloys can be used in the hot sections of gas turbine engines, e.g., burner cans, and in industrial applications where aggressive corrosives are encountered, e.g., molten glass, flue dust, fly ash, etc.

According to the invention, alloys exhibiting high resistance to oxidation at temperatures as high as 1300°C have the compositions set forth in claim 1.

Generally speaking, the present invention contemplates dispersion strengthened powder metallurgically produced iron-chromium-aluminum alloys containing from 20 to 30% chromium, e.g. at least 22.5% Cr, and 5 to 8% aluminum. Where flat rolled products are required, e.g., sheet, for intended uses in which a significant degree of fabricability is necessary, the aluminum content should not exceed 6.25% i.e. the aluminum should be from 5% to 6.25%. Advantageously, in this regard, the chromium should be from 23 to 27% and the aluminum from 5 to 6%. The alloys may also contain up to 5% titanium, up to 2% each of zirconium, hafnium, tantalum and venadium, up to 6% each of molybdenum and tungsten, up to 0.5% each of silicon and niobium, up to 0.05% each of calcium, yttrium and rare earth metals, up to 0.2% boron and the balance, apart from impurities, iron plus, to enhance strength, a small but effective amount, e.g., 0.2 volume %, of at least one finely divided dispersoid having a melting point of at least about 1510°C (2750°F) and selected from the group consisting of oxides, nitrides, carbides, borides and other refractory materials. In this connection oxides may be present up to about 10 volume % whereas carbides should not exceed about 2 volume %. Nitrides and borides need not exceed 5% by volume.

In carrying the invention into practice, the chromium content should not exceed 30% to minimize the formation of deleterious levels of topologically close packed (TCP) phases such as sigma, phases which adversely impact mechanical properties. Given cost, there is no significant benefit derived with chromium percentages above about 27%. Reducing the percentage of chromium below 20% gives rise to the risk that oxidation resistance will be decreased at a given aluminum level.

Aluminum should be from 5% to 8% for oxidation and corrosion resistance but as indicated, supra, preferably should not exceed 6% when seeking the optimum in terms of fabrication into sheet, strip, etc. Such elements as nickel and cobalt are not required and confer no particular advantage. Carbon need not exceed 0.1% though higher percentages can be tolerated. Our investigation has not shown silicon or boron to be particularly beneficial. Boron is thought to be causative of (or a contributor to) distortion when the sheet product form is heat treated at elevated temperatures. It preferably should not exceed 0.1%. Such constituents as titanium, zirconium, tantalum, niobium, hafnium, zirconium and vanadium need not exceed 1%. Tantalum, for example, at the 1% level has resulted in a loss of fabricability. It tends to stiffen the alloys of the invention and possibly raises the ductile-brittle trans-formation temperature too much. A range of titanium from 0.2 or 0.25 to 0.75% is preferred.

The alloys of the invention are most preferably produced by mechanical alloying as described in U.S. 3,992,161, although other dispersoid strengthening powder metallurgy processes may be employed.

To give those skilled in the art a better understanding of the invention the following information and data are presented.

A series of alloy compositions were prepared using raw material powders namely, elemental (e.g., Fe, Cr, Al), master alloy (e.g., Fe-Cr-Al-Ti) and yttrium bearing oxide (Y₂O₃) which powders were thereafter blended to produce the chemistries given in Table I, in which Alloys H and I are in accordance with the invention but the others are not. The powder blends were mechanically alloyed (MA) in high energy ball mills under an argon atmosphere for about 24 hours at a ball-to-powder ratio of about 20:1 using steel balls as the impacting/grinding media. The MA powders were screened to remove the coarser particles (above about 600 microns), placed in mild steel cans, sealed and hot compacted by extrusion. The extrusions were decanned and then hot and cold rolled to 1.25 mm (0.05in) thick sheet, the sheet thereafter being subjected to a final anneal which was typically 1315°C (2400°F) for 1 hour to achieve recrystallization.

Standard size specimens were cut from the sheets produced and the ground to approximately 600 grit for use in accelerated oxidation tests. Cyclic oxidation testing was used and this consisted of exposing samples at temperatures of 1200°C, 1250°C and 1300°C in air + 5%H₂O for 24 hour cycles, then cooling to room temperature and weighing. Results are reported in Tables II and III.

In Table III below the times from initiation of accelerated oxidation to completion are reported:

An examination of the data in Table II and III reflects that increasing the chromium level from 16% to 20% resulted in some improvement in oxidation resistance at a constant aluminum level, Alloy A vs. Alloys B and C, the results being quite poor at the 1300°C test temperature. However, raising the chromium level to 23.5%, Alloy D, did not manifest any significant improvement, particularly at the 1300°C test condition.

Alloys B, and C are representative of a typical '161 composition, i.e., 20% Cr/4.5% Al. At 1300°C, the initiation of accelerated oxidation to the point of completion spanned but 2 days. See Table III. Increasing the chromium content to 24% reduced in half the rate of accelerated oxidation (Alloy D, Table III) and increasing the aluminum level from 4.5 to 6.5% to give an alloy in accordance with the invention again markedly reduced the rate of attack (Alloy H, Table III). This pattern of behavior is of practical importance because a significant reduction in the rate of attack may extend service life to allow a repair operation and, thus, avoid the consequences of a catastrophic failure.

Figures 1-3 illustrate more graphically what happens by increasing the chromium level of a typical commercial '161 alloy which contained, apart from the different chromium levels, 0.02%/wt C, 4.5%/wt Al, 0.3%/wt. Ti, 0.5%/vol. Y₂O₃, incidental impurities, with iron being essentially the balance. At each test temperature of 1200°C, 1250°C and 1300°C, the spallation rate (mass change) was greater in respect of the higher percentage of chromium. In accordance with the subject invention, the aluminum content should also be increased, preferably proportionately, to reduce the rate of spallation and ensure better integrity of the alloy composition. This is reflected by Figures 4 and 5 where at a 25% Cr level the spallation rate is markedly reduced through the co-presence of an additional 2% of aluminum above the '161 alloy.

A further practical advantage of the alloys of our invention is that they are deemed to afford improved high temperature oxidation and corrosion resistance in thin gauges in comparison with prior art material. Sheet thickness, for example, of 1.25 mm (0.05 in.) are typical for the 20% Cr/4.5% Al '161 alloy as commercially produced. In such gauge section there is a propensity to undergo accelerated oxidation attack early on for lack of, comparatively speaking, bulk concentration of aluminum and chromium atoms available for surface (oxide) protection. Put another way, such accelerated attack can cause pitting, pitting which will penetrate through, for example, sheet. Alloys of the invention offer a higher concentration of reserve aluminum and/or chromium atoms.

With regard to fabricability Figure 6 depicts a general correlation between chromium and aluminum in respect of their combinative effect on bendability, a criterion used to assess fabricability. In this connection, sheet specimens approximately 1.3 mm (0.05 in) (1 t) thick, 1.27 mm (1/2 in) in width and about 5-10 cm (2 to 4 in) in length were bent over a rod of approximately 1.6 mm (0.1 in) thick (2 t). Tests were made in both the longitudinal and transverse directions. The black shaded area is indicative that some cracking was evident from the tests. As can be seen, the standard '161 alloy of 20% Cr/4.5% Al is quite fabricable. But at a 30% Cr/4.5% Al level cracking was experienced. Some cracking was noted in the transverse direction with an alloy of approximately 19% chromium and 5.2% aluminum. The alloy containing 6.6% aluminum and about 25% chromium cracked excessively in the transverse direction, the bend angle being less than 50° versus a desired 105° or more. For purposes of fabricability the aluminum content, as noted above herein, advantageously should not exceed 6% and more preferably is not above 5.75%.

Apart from flat rolled products, the alloys contemplated herein can be used in hot worked and/or machined bar and other mill product shaped forms including forgings and tubing. It may be cost effective, for example, to machine components from bar for, say, flame guides or glass extrusion dies.

Although the present invention has been described in conjunction with preferred embodiments, it is to be understood that the invention is not limited to these embodiments.

## Claims

1. A powder metallurgical iron-chromium-aluminium dispersion strengthened alloy exhibiting high resistance to oxidation at temperatures as high as 1300°C and consisting of 20 to 30%/wt. chromium, 5 to 8%/wt. aluminum, an amount from 0.2 to 10% by volume of a refractory dispersoid effective to enhance strength and selected from the group consisting of oxides, carbides, nitrides and borides, with or without one or more of the following additional constituents: up to 5%/wt. titanium, up to 2%/wt each of zirconium, hafnium, tantalum and vanadium, up to 6%/wt each of molybdenum and tungsten, up to 0.5%/wt. silicon, up to 0.5%/wt. niobium, up to 0.05%/wt. each of calcium, yttrium and rare earth metals, up to 0.2%/wt boron, the balance, apart from impurities, being iron.

2. An alloy according to claim 1 containing at least 22.5% chromium.

3. An alloy according to claim 1 or claim 2 containing from 0.25 to 0.75% titanium.

4. A powder metallurgical iron-chromium-aluminum dispersion strengthened alloy in the form of a flat rolled product such as sheet and strip characterised by good fabricability and resistance to oxidation at temperatures as high as 1300°C, said product being formed from an alloy according to any preceding claim in which the chromium content is at least 23%/wt. and the aluminum content is from 5 to 6.25%/wt.

5. An alloy product according to claim 4 wherein titanium is present in an amount from 0.2 to 0.75%/wt.

6. An alloy product according to claim 4 or claim 5 in which the aluminum content does not exceed 6%/wt.

7. An alloy product according to any one of claims 4 to 6 in which the chromium content is from 23 to 27%/wt.

8. An alloy product according to any one of claims 4 to 7 in which the refractory dispersoid is one or more oxides in an amount up to 10 volume %, carbides up to 2 volume %, nitrides up to 5 volume % and borides up to 5 volume %, all percentages being of the total volume of the alloy.

9. A metal component for the hot stage section of an aircraft gas turbine engine, formed from an alloy product according to any one of claims 4 to 8.

10. A metal component according to claim 9 in the form of a burner can.

11. An alloy product according to any one of claims 4 to 9 wherein the powder is produced by mechanical alloying.

## Patentansprüche

1. Pulvermetallurgisch hergestellte dispersionsgehärtete Eisen-Chrom-Aluminium-Legierung mit hoher Oxydationsbeständigkeit bei Temperaturen bis 1300°C aus 20 bis 30 Gew.-% Chrom, 5 bis 8 Gew.-% Aluminium, 0,2 bis 10 Vol.-% eines schwerschmelzbaren, die Festigkeit erhöhenden Dispersoids aus der Gruppe der Oxyde, Karbide, Nitride und Boride sowie fakultativ einzeln oder nebeneinadnder bis 5 Gew.-% Titan, jeweils bis 2% Zirkonium, Hafnium, Tantal und Vanadium, jeweils bis 6 Gew.-% Molybdän und Wolfram, bis 0,5 Gew.-% Silizium, bis 0,5 Gew.-% Niob, jeweils bis 0,05 Gew.-% Kalzium, Yttrium und Seltene Erdmetalle sowie bis 0,2 Gew.-% Bor, Rest abgesehen von Verunreinigungen Eisen.

2. Legierung nach Anspruch 1 mit mindestens 22,5% Chrom.

3. Legierung nach Anspruch 1 oder 2 mit 0,25 bis 0,75% Titan.

4. Pulvermetallurgische, dispersionsgehärtete Eisen-Chrom-Aluminium-Legierung in Gestalt eines gewalzten Flachprodukts wie Blech und Band mit guter Verarbeitbarkeit und Oxydationsbeständigkeit bei Temperaturen bis 1300°C aus einer Legierung nach einem der Ansprüche 1 bis 3, deren Chromgehalt mindestens 23 Gew.-% und deren Aluminiumgehalt 5 bis 6,25 Gew.-% beträgt.

5. Legierungsprodukt nach Anspruch 4, dessen Titangehalt 0,2 bis 0,75 Gew.-% beträgt.

6. Legierungsprodukt nach Anspruch 4 oder 5, dessen Aluminiumgehalt 6 Gew.-% nicht übersteigt.

7. Legierungsprodukt nach einem der Ansprüche 4 bis 6, dessen Chromgehalt 23 bis 27 Gew.-% beträgt.

8. Legierungsprodukt nach einem der Ansprüche 4 bis 7 mit einem schwerschmelzbaren oxydischen Dispersoid in einer Menge bis 10 Vol.-%, bis 2 Vol.-% Karbiden, bis 5 Vol.-% Nitriden und bis 5 Vol.-% Boriden, jeweils bezogen auf das Gesamtvolumen der Legierung.

9. Metallkomponente für den Heißbereich einer Flugzeuggasturbine aus einem Legierungsprodukt nach einem der Ansprüche 4 bis 8.

10. Metallkomponente nach Anspruch 9 in Gestalt einer Brennerbüchse.

11. Legierungsprodukt nach einem der Ansprüche 4 bis 9, bei dem das Pulver durch mechanisches Legieren hergestellt worden ist.

## Revendications

1. Un alliage en poudre fer-chrome-aluminium renforcé par dispersion produit par métallurgie présentant une résistance élevée à l'oxydation à des températures pouvant aller jusqu'à 1300°C et consistant en de 20 à 30% en poids de chrome, de 5 à 8% en poids d'aluminium, une quantité allant de 0,2% à 10% en volume d'un système colloïdal à grande dispersion réfractaire efficace pour accroître la solidité et choisi dans le groupe consistant en les oxydes, les nitrures, les carbures et les borures, avec ou sans un ou plusieurs des constituants supplémentaires suivants : jusqu'à 5% en poids de titane, jusqu'à 2% en poids chacun de zirconium, d'hafnium, de tantale et de vanadium, jusqu'à 6% en poids chacun de molybdène et de tungstène, jusqu'à 0,5% en poids de silice, jusqu'à 0,5% en poids de niobium, jusqu'à 0,05% en poids chacun de calcium, d'yttrium et de métaux terreux rares, jusqu'à 0,2% en poids de bore et le restant, exception faite des impuretés, étant du fer.

2. Un alliage selon la revendication 1 contenant au moins 22,5% de chrome.

3. Un alliage selon la revendication 1 ou la revendication 2 contenant de 0,25 à 0,75% de titane.

4. Un alliage en poudre fer-chrome-aluminium renforcés par dispersion produit par métallurgie sous la forme d'un produit laminé à plat tel qu'une feuille et une bande caractérisé par une bonne fabricabilité et résistance à l'oxydation à des températures allant jusqu'à 1300°C, ledit produit étant formé à partir d'un alliage selon l'une quelconque des revendications précédentes dans lequel la teneur en chrome est d'au moins 23% en poids et la teneur en aluminium va de 5 à 6,25% en poids.

5. Un produit en alliage selon la revendication 4 dans lequel le titane est présent en une quantité qui va de 0,2 à 0,75% en poids.

6. Un produit en alliage selon la revendication 4 ou la revendication 5 dans lequel la teneur en aluminium ne dépasse pas 6% en poids.

7. Un produit en alliage selon l'une quelconque des revendications 4 à 6 dans lequel la teneur en chrome va de 23 à 27% en poids.

8. Un produit en alliage selon l'une quelconque des revendications 4 à 7 dans lequel le système colloïdal à grande dispersion réfractaire est un ou plusieurs oxydes en une quantité allant jusqu'à 10% en volume, carbures jusqu'à 2% en volume, nitrures jusqu'à 5% en volume et borures jusqu'à 5% en volume, tous les pourcentages étant par rapport au volume total de l'alliage.

9. Un composant métallique pour la section de l'étape chaude d'un moteur d'avion à turbine à gaz, formé à partir d'un produit en alliage selon l'une quelconque des revendications 4 à 8.

10. Un composant métallique selon la revendication 9 sous la forme d'un brûleur.

11. Un produit en alliage selon l'une quelconque des revendications 4 à 9 dans lequel la poudre est produite par alliage mécanique.
